

83

Patented Mar. 7, 1933

1,900,211

## UNITED STATES PATENT OFFICE

JOSEPH RIGBY WATSON, OF SAN FRANCISCO, CALIFORNIA, ASSIGNOR TO VIRGINIA LOUISE WATSON, OF SAN FRANCISCO, CALIFORNIA

## FIRE RESISTANT AND PRESERVATIVE COMPOSITION

No Drawing.

Application filed July 18, 1928. Serial No. 293,784.

166-82

My invention relates to a fire resistant and preservative composition, and particularly one which serves as a coating composition.

An object of my invention is the provision of a composition of the character described which will effectively act as a preservative coating for materials to which it is applied.

Another object of my invention is the provision of a composition of the character described which serves as a fire resistant coating for combustible materials.

My invention possesses other objects and valuable features, some of which will be set forth in the following description of my invention. It is to be understood that I do not limit myself to the showing made by the said description, as I may adopt varying forms of my invention within the scope of the claims.

20 In terms of broad inclusion my invention comprises a mixture of an alkali metal silicate, an alum or other equivalent salt, and a fluorine compound of the character of cryolite or of an alkali metal fluosilicate, in a vehicle 25 such as a mineral oil, bituminous material such as tars and asphalts, or drying oils such as linseed oil. This mixture provides a coating composition which can be applied to the materials to be treated.

30 In terms of greater detail, a satisfactory composition has been prepared by the mixture of the following substances in approximate parts by weight:

|                 | Parts |
|-----------------|-------|
| Cryolite        | 4     |
| Ammonia alum    | 2     |
| Sodium silicate | 2     |

The ingredients in powdered form are thoroughly mixed and incorporated in a non-aqueous vehicle such as tung oil, linseed oil, mineral oil, or a bitumen such as soft asphalts or tars. Although any of these vehicles are satisfactory, the bituminous vehicle is preferred. The amount of vehicle used depends 45 to a great extent upon the viscosity of the

final mixture; therefore, it is apparent that various volumes of vehicle can be employed. However, for a mixture which can be applied with a brush, from 2 to 3½ gallons of vehicle are preferred when the parts of the other ingredients are in pounds.

For the cryolite in the above composition, satisfactory results have been obtained by substituting the same quantity of an alkali metal fluosilicate such as sodium or potassium <sup>50</sup> fluosilicate. Sodium fluosilicate is preferred due to its greater availability and lesser cost. Also a mixture of various quantities of cryolite and an alkali metal fluosilicate can be used in place of one of these compounds alone <sup>55</sup> to give a total of four parts by weight of fluorine compound. Ammonia alum is preferred since the best results have been obtained by its use, but various other alums can be substituted therefor. For instance the <sup>60</sup> same quantity of ammonia chrom. ammonia iron, potassium, sodium, or potassium iron alums can be employed; or if desired straight salts such as ferric or ferrous sulfate, or aluminum sulfate can be substituted for the <sup>65</sup> two parts of alum. In place of the sodium silicate, the same quantity of another alkali metal silicate as potassium silicate can be used.

The proportions stated in the preceding <sup>70</sup> example are those which have been found to produce the best results. However, the quantities of the ingredients or their substitutes, may be varied within a wide range with satisfactory results. For example, the <sup>75</sup> following range of substances in parts by weight can be employed with the vehicles previously described:

|                                                                                                         | Parts   |
|---------------------------------------------------------------------------------------------------------|---------|
| <u>Fluorine compound</u> of the character of <u>cryolite</u> or of an <u>alkali metal fluo-silicate</u> | 85      |
| <u>An alum</u> or the equivalent                                                                        | 1 to 10 |
| <u>Alkali metal silicate</u>                                                                            | 1 to 5  |

The quantity of vehicle is determined by the <sup>90</sup>

final viscosity desired. As previously pointed out, it is preferred to use a volume of vehicle which will provide a coating that can be readily applied by means of a brush. 5 However, the quantity can be adjusted to suit various needs.

In preparing these compositions, the finely divided compounds are thoroughly incorporated in the desired vehicle by mixing and 10 stirring.

The compositions when applied as a coating to combustible materials such as wood, paper, or fabrics such as canvas, serve to resist fire for a long time, and to prevent 15 the spreading of flames. The materials thus treated will only char at the point of contact with the fire without bursting into flames. It is thought that this condition is created by the generation of gases which 20 prevent the access of oxygen to the treated material. As previously set forth, it is preferred to apply the coating by means of a brush. However, if desired, the materials to be treated may be immersed in a bath of the 25 coating composition.

Not only have these compositions been found to effectively resist fire, but they also act as preservatives when applied to materials such as wood, railroad ties, or wood 30 pilings.

I claim:

1. A fire resistant and preservative composition comprising a substance of the group consisting of cryolite and an alkali metal 35 fluosilicate, an alkali metal silicate, and an oil vehicle.

2. A fire resistant and preservative composition comprising a substance of the group consisting of cryolite and an alkali metal 40 fluosilicate, an alum, an alkali metal silicate, and a bituminous vehicle.

3. A fire resistant and preservative composition comprising a vehicle, and the following substances in parts by weight:

45 4. A substance of the group consisting of cryolite and an alkali metal fluosilicate 1 to 10  
An alum 1 to 4  
50 An alkali metal silicate 1 to 5

55 5. A substance of the group consisting of cryolite and an alkali metal fluosilicate 4  
An alum 2  
An alkali metal silicate 2

60 6. A fire resistant and preservative composition comprising cryolite, sodium silicate, and an oil vehicle.

65 7. A fire resistant and preservative composition comprising cryolite, sodium silicate, an alum, and a vehicle.

7. A fire resistant and preservative composition comprising cryolite, sodium silicate, and alum, and a bituminous vehicle.

8. A fire resistant and preservative composition comprising a bituminous vehicle, and 70 the following substances in parts by weight:

|                 | Parts     |
|-----------------|-----------|
| Cryolite        | 1 to 10   |
| An alum         | 1 to 4    |
| Sodium silicate | 1 to 5 75 |

9. A fire resistant and preservative composition comprising a bituminous vehicle, and the following substances in approximate parts by weight:

|                 | Parts |
|-----------------|-------|
| Cryolite        | 4     |
| An alum         | 2     |
| Sodium silicate | 2     |

10. A fire resistant composition comprising 85 a substance of the group consisting of cryolite and an alkali metal fluosilicate, an alkali metal silicate, and a bituminous vehicle, the alkali metal silicate and substance being in such proportions as to efficaciously protect 90 against fire.

11. A fire resistant composition comprising 95 a substance of the group consisting of cryolite and an alkali metal fluosilicate, a metal sulfate, and a bituminous vehicle, the metal sulfate and substance being in such proportions as to efficaciously protect against fire.

In testimony whereof, I have hereunto set my hand.

JOSEPH RIGBY WATSON. 100

100

105

110

115

120

125

130